

A. SCHWARZ.  
ORE CONCENTRATING METHOD.  
APPLICATION FILED JAN. 17, 1917.

1,237,961.

Patented Aug. 21, 1917.



INVENTOR  
Alfred Schwarz  
BY  
H. F. Bryant  
ATTORNEY

# UNITED STATES PATENT OFFICE.

ALFRED SCHWARZ, OF JOPLIN, MISSOURI, ASSIGNOR TO METALS RECOVERY COMPANY, OF NEW YORK, N. Y., A CORPORATION OF MAINE.

## ORE-CONCENTRATING METHOD.

1,237,961.

Specification of Letters Patent. Patented Aug. 21, 1917.

Application filed January 17, 1917. Serial No. 142,917.

To all whom it may concern:

Be it known that I, ALFRED SCHWARZ, a subject of the Emperor of Germany, residing at Joplin, in the county of Jasper and 5 State of Missouri, have invented certain new and useful Improvements in Ore-Concentrating Methods, of which the following is a specification.

Heretofore ores and metalliferous substances have been separated into their constituents, that is, metal or mineral portions from the gangue by means of the well known affinity therefor of certain oily or similar hydrocarbons or hydrocarbon mixtures, or 10 resinous or other similar selective agents by agitating the ore pulp and water with air and forming a foam or froth, such froth carrying the metalliferous substances to the surface of the water, whereafter such mineral particles carried with the froth were separated from the pulp and the water and gangue by skimming, overflowing and similar means. Air, however, is an oxidizing agent and in some cases acts destructively 15 upon the hydrocarbon used and the great quantities of air forced through the solution volatilize a certain portion of the hydrocarbon. Furthermore, air in no wise benefits the process other than as a lifting agent. 20 Whereas, during a series of experiments, I have found that gases other than air are sometimes more closely related to the ingredients, and when intended to act upon the mineral or gangue content of the ore, will 25 benefit the process of flotation. It has been suggested heretofore, and I have mentioned it in one of my previous patents Number 807,502, dated December 19, 1905, to generate gas within the pulp as a means of increasing the buoyancy of the mixture of mineral and oil, but in all cases air was admitted, thus eliminating complete control over 30 the type of gases to be used.

It is the object of the present invention to 45 permit the concentration of mineral by the use of solid or liquid hydrocarbon and gases or resinous or other similar selective agents, without the influence of the component parts of the air. The type of gases to be used may 50 be different in the treatment of different ores and with the use of different hydrocarbon, or other selective agent. There may be also mixtures of gases used according to the chemical effects desired. In some cases it 55 may be desirable to use an unfixed-gas ca-

pable of complete or partial condensation. In the process itself, volatile portions of the hydrocarbon, or other selective agent, used are carried constantly through the ore pulp and are so-caused to act continually upon the 60 ore, whereas, in the previous methods such volatile portions were carried out through the air and lost. In the foregoing description, when I refer to hydrocarbon I not only mean to include compounds which are composed exclusively of hydrogen and carbon, but also hydrocarbon derivatives and compounds, and resins and other agents which are sometimes classed among the hydrocarbons. Illustrating the process in a specific 65 case I will give the following example:

In one of my previous patents, Number 807,501, dated December 19, 1905, I have described the conversion of carbonate and oxids of metals into sulfids or the surface 70 coating of the same by means of the use of soluble sulfids, and in practice I have used hydrogen sulfid gas to cause the said conversion. I have found, however, that the presence of excessive quantities of air sometimes renders the process difficult to carry 75 out, whereas, when the air is excluded from the operation and either hydrogen sulfid gas or a mixture of hydrogen sulfid gas and other gases is used, this will not only eliminate the detrimental action of the air agitation or of air otherwise carried into the process, but will enable the operator to control certain chemical re-actions beneficial to 80 the said process.

In carrying out my invention I may use any one of the known flotation machines sealing the same, however, against the atmospheric air thus permitting only such gas mixtures as may be desired in the treatment, to enter the flotation cell by suitable means at will of the operator. In this manner I may use in connection with the flotation cell one or more gas receivers, suitable pumping devices to circulate the gas in the 100 system, and taking the excess gas used in the cell, and pumping same back into a receiver or in any other portion of the circuit where same may be desired. It is obvious of course, that in this manner any 105 volatile portions of the oils or hydrocarbon mixtures used will be retained within the closed circuit and in re-using the gas will re-enter the system and in this manner a considerable saving and preservation of the 110

character of the hydrocarbon will take place.

To illustrate the process I have shown in the annexed drawing an ordinary ore flotation machine modified to carry out my process. In the drawing similar reference characters refer to corresponding parts throughout the several views, Figure 1 thereof being a central vertical section of the machine, parts being shown in elevation; and Fig. 2 is a top plan view thereof with the main cover member removed.

The machine comprises two tanks 1-1 designed to receive the concentrate and a tank 2, arranged therebetween, designed to receive the tailings. These three tanks may only contain a small proportion of the product submerged in water. A constant water level is maintained in these tanks thus acting as a water seal against the escape of the gases. On the rear of the machine is attached what is known as a Pachuca tank, 3, serving to agitate the mixture with the gas, and properly distributing the hydrocarbon and gas through the pulp. The pulp is charged into the Pachuca tank from the storage tank 17, through the pipe 18, controlled by the valve 19, so that this again forms a water seal against the escape of the gas. It is, of course, understood that the Pachuca tank is closed on the top. Escaping gases from this tank go through the passage 4, and are collected at 14 by the suction of the pump. The over flow from the Pachuca tank enters into the flotation cell through the passage 4, which is air tight, into the hopper 5, which feeds the mixture into the bottom of the cell. At 6-6-6-6 are arranged valves to regulate the gas as it enters the cell and percolates upwardly through the porous bottom 7 into the ore pulp emerging from the same on the surface carrying with it the mineral particles coated with the hydrocarbon. These mineral particles overflow through the launders 8 and 8 into tanks 1 and 1 where two water sprays, 9 (only one being shown), serve to break down the gas bubbles and precipitate the mineral particles into the bottom of the tank below the water level shown at 10, from where they may be drawn off through the valved outlet 11. The gangue or tailings will enter through the passage 12 into the central compartment 2 where enough water and tailings are stored to form a water seal against the escape of the gases. The entire machine is closed by the cover 13 and at 14 a pipe connection leads the escaping gases from the Pachuca tank, the flotation cell proper, and the storage tanks 1, 1 and 2, back to the pump 15, as indicated by the arrows in Fig. 1 of the drawing, from thence it passes through the gas receiver 16, and through the porous bottom 7 by way of the valved connections 6.

What I claim as my invention and desire to secure by Letters Patent is:

1. A flotation process for concentrating ores, said process consisting in charging a body of ore pulp containing modifying agents, with a bubble-producing gas, other than air; substantially excluding atmospheric air from contact with the ore mixture and gas; withdrawing the liberated gas from above the pulp mass; and directly re-delivering said gas throughout the area of the pulp mass.

2. A flotation process for concentrating ores, said process consisting in charging a body of ore pulp containing modifying agents, with a bubble-producing gas, other than air; substantially excluding atmospheric air from contact with the ore mixture and gas; removing the floated metalliferous particles of the ore mass by the expelling action of the progressively rising bubbles below; withdrawing the liberated gas from above the pulp mass; and directly re-delivering said gas throughout the area of the pulp mass.

3. A flotation process for concentrating ores, said process consisting in charging a body of ore pulp containing a modifying agent with a bubble producing agent other than air; substantially excluding atmospheric air from contact with the ore mixture and bubble producing agent; withdrawing liberated gas from a bubble-breaking-down region above the pulp mass; and directly re-delivering said gas throughout the area of the pulp mass while maintaining the exclusion of air from said mass.

4. A flotation process for concentrating ores, said process consisting, essentially, in gasifying a body of ore pulp to cause bubbles to form and rise through said body and carry the mineral particles thereof to the surface; excluding atmospheric air from contact with the ore mixture and gasifying agent during the gasifying of the pulp; withdrawing liberated gas from above the pulp mass; and directly re-delivering said gas throughout the area of the pulp mass.

5. A flotation process for concentrating ores, said process consisting in mixing ore with a hydrocarbon and gas substantially under the exclusion of atmospheric air; and producing in the mixture bubbles capable of carrying the mineral particles of the mass to the surface thereof, and separating the bubbles; precipitating the mineral particles from the bubbles into water; and drawing off the gases from the flotation and the froth-breaking-down regions and re-injecting said gases into the ore mixture.

6. A flotation process for concentrating ores, said process consisting in charging a body of ore pulp containing modifying agents, with a gas, other than air; substantially excluding atmospheric air from

- contact with the ore mixture and gas during the gasifying of the pulp; charging the ore mass with additional bubble-producing gas, other than air, while maintaining the exclusion of atmospheric air therefrom and from the ore mass; withdrawing the liberated gas from above the pulp mass; and directly redelivering said gas throughout the area of the pulp mass.
- 10 7. A flotation process for concentrating ores, said process consisting in charging a body of ore pulp containing modifying agents, with a gas, other than air; substantially excluding atmospheric air from contact with the ore mixture and gas; charging the ore mass with additional bubble-producing gas, other than air, while maintaining the exclusion of atmospheric air therefrom and from the ore mass; removing the floated metalliferous particles of the ore mass by the expelling action of the progressively rising bubbles below; precipitating the mineral particles from the bubbles in a sealed chamber and maintaining a liquid seal in said chamber; withdrawing the liberated gas from above the pulp mass; and re-delivering said gas as bubbles throughout the area of the pulp mass.
- 15 8. A flotation process for concentrating ores, said process consisting, essentially, in including a flotation chamber in a circuit closed to the admission of atmospheric air; gasifying ore pulp in said chamber while excluding atmospheric air from contact with the ore mixture and gasifying agent; drawing off liberated gases from the bubble-breaking-down region of the flotation chamber; and directly redelivering said gases into the ore mixture throughout the area thereof.
- 20 9. A flotation process for concentrating ores, said process consisting, essentially, in including a flotation chamber in a circuit closed to the admission of atmospheric air; gasifying ore pulp in said chamber while excluding atmospheric air from contact with the ore mixture and gasifying agent; drawing off liberated gases from the bubble-breaking-down region of the flotation chamber; and directly redelivering said gases into the ore mixture throughout the area thereof.
- 25 8. A flotation process for concentrating ores, said process consisting in charging a

In testimony whereof I affix my signature. 55  
ALFRED SCHWARZ.